

Aug. 27, 1935.

D. V. EDWARDS ET AL

2,012,339

RECTIFIER

Filed Jan. 7, 1931

*Fig. 1.*



*Fig. 2.*



INVENTORS

*Donald V. Edwards*  
*Earl R. Smith*

BY their ATTORNEYS

*Edwards, Bower & Pool*

## UNITED STATES PATENT OFFICE

2,012,339

## RECTIFIER

Donald V. Edwards, New York, N. Y., and Earl K. Smith, East Orange, N. J., assignors to Electrons, Inc. of Delaware, a corporation of Delaware

Application January 7, 1931, Serial No. 507,052

8 Claims. (Cl. 250—27.5)

This invention relates to controlled rectifiers of the gaseous type.

The object of the invention is to provide means for preventing loss of grid control.

5 Heretofore in tubes of this type, after the tube has been in operation for a short time it has occurred that the tube started despite the fact that the grid voltage was more negative than the trigger voltage.

10 The invention will be described with reference to the accompanying drawing, in which

Fig. 1 shows a conventional rectifier embodying the invention; and

Fig. 2 an enlarged portion of a part of the grid structure embodying the invention.

15 In applicants' Patent No. 1,905,692 issued April 25, 1933, the structure of an electron tube of the type shown in Fig. 1 of the present application is described and claimed.

20 1 represents the glass tube; 2 the plate; 4 the cathode, and 8 the grid. In the form shown the cathode 4 is in cylindrical form having a plurality of filaments 3 connected to the filament circuit 5. Preferably the filaments 3 are oxide coated but the interior of the cylinder or both cylinder and filaments may be oxide coated. As a coating we prefer the resultant product of an alkaline earth oxide and an oxide of a metal capable of forming amphoteric compounds less acid 25 than titanic acid, such, for example, as aluminum oxide, zirconium oxide or the like, heated in vacuum.

30 As gaseous conducting medium we prefer argon, although mercury or other gas or mixtures thereof may be employed.

35 The grid structure shown comprises a disk 8 having an opening therein across which are a number of bars 10, the spaces 9 between the bars being suitably adjusted. Plate 2 and cathode 4 are connected by circuit 6 receiving power from an alternating current source 1 through transformer 11. Preferably the potential on the grid is controlled by a potentiometer 15 connected across the terminals of a battery 18 through a 40 limiting resistance 17, and a variable pointer 16 whereby the battery voltage upon the grid may be adjusted. The battery 18 is connected to the cathode through the secondary 20 of a transformer connected across the plate-cathode circuit 45 and thence through wire 19 to the cathode. Thereby an alternating potential which may be made out of phase by the insertion of a condenser 21, or an inductance 22 or both, is also applied to the grid.

50 55 The tube herein described is typical, inasmuch

as in practice the various parts of the circuit in which the tube is used will assume various shapes, proportions and arrangements.

The loss of control above referred to, in our opinion is caused by cold emission of electrons from the grid when barium evaporated from the filament is deposited on the grid; that the positive electrostatic field from the plate pulls these electrons from the grid; and that these electrons on their way to the plate ionize the gas and the 10 tube then starts in spite of a negative charge on the grid.

Various expedients have been proposed with a view to minimizing the chances of barium so depositing. One of such proposals was to reduce 15 the current density through the tube, thereby to reduce the possible barium vaporization. We propose to provide means for preventing emission from the grid even though barium be deposited thereon.

20 To this end we employ a poisonous grid coating, thereby to permit increased density of the current through the tube and the use of a smaller grid, and thereby decreasing the relative heating of the grid, even though the tube be operated at 25 increased current density. We further provide means for maintaining the grid in the poisoned condition for a prolonged time.

In one embodiment of the invention the grid is 30 coated with the oxide of a metal of high work function, for example the oxides of tantalum, molybdenum and tungsten. The body of the grid may be of other material but preferably is a metal of high work function such as tungsten.

In Fig. 2 the oxide coating is conventionally 35 shown at 25 on the grid wires 10. To avoid peeling off of the oxide, if tungsten oxide is used, we prefer to use the oxide in amorphous form, instead of the crystal formation customarily used. One way of converting the crystalline formation 40 into the amorphous form is to treat it with ammonia at a lower temperature than minus 21° centigrade.

The effect of heat radiated from the filament, heat radiated from the discharge and ionic bombardment should be kept below the temperature of chemical breakdown of the oxide. Thus the current density through the tube may be largely increased beyond present practice. This permits the use of a smaller grid than normally used, and 50 in turn reduces the quantity of heat received by the grid and reduces the distance the heat has to flow to reach the heat radiating part of the grid outside of the discharge. In practice we have found it possible to build tubes having more 55

than ten times the current density through the grid than in prior tubes. This has made possible a grid having one-tenth of the former grid surface and consequent reduction in grid heat. A 5 tube of medium size, following the former practice, would require, say, ten or more square inches of grid surface, whereas with our method this has been cut to one square inch. The temperature of the discharge is extremely high regardless 10 of the current density and therefore the heat received by the smaller grid will be about one-tenth that of the other. Furthermore, this much smaller quantity of heat has only to flow through at the most one-half inch of grid wire to reach 15 the heat radiating part of the grid outside of the discharge, whereas with the large grid it would have to flow through at least one and one-half inches of metal. The result of this is that the small high current density grid runs only a few 20 degrees above the heat radiating portion of the grid. When the grid is large the heat gradient must be high, and therefore the center becomes very hot.

Regarding materials for poisoning the barium, 25 we have tried oxides of tantalum, molybdenum and tungsten and have found them satisfactory. We have reason to believe, however, that the oxides of all high work function but nonradio active materials will work satisfactorily. In fact, 30 some measurements show that some of the oxides of metals whose oxides are anhydrides of amphoteric compounds, particularly the more highly negative ones, would be satisfactory. We also find that carbides, nitrides and halogen compounds 35 of high work function nonradio active metals will work satisfactorily.

Since there is a tendency for the filament to 40 continue sending barium atoms to the grid, we have found it advantageous to provide a means for feeding poisoning material to the grid during the operation of the tube. To this end the plate 45 is made of carbon, which, when the tube is in operation, will occasionally release, by disintegration, carbon ions. These carbon ions will be attracted to the grid by the electrostatic field in the same manner as the barium atoms are attracted 50 from the cathode to the grid and will deposit on top of such barium atoms as may have reached the grid, and will poison any emission of electrons from the grid. If the tube is so arranged as to have a continuous disintegration of carbon it is possible to poison the barium atoms by freshly deposited carbon atoms about as fast as barium 55 deposits on the grid.

Carbon alone is not poisonous any more than 60 any equally electro-negative metal, but due to its peculiar absorbing powers it always contains considerable quantities of absorbed gases and impurities which are never completely removed on the pump and which serve to poison the barium deposited on it. After the tube has been in operation some time, however, these impurities are gradually cleaned from the surface and pure carbon is exposed, after which the tube loses control. 65 But when the carbon ions are released from the plate by disintegration as above described the carbon is deposited on top of the barium and effectively poisons emission from the barium.

We offer the following as a theoretical explanation of the effectiveness of the oxides of high work function elements, and the depositing of carbon ions on the oxides, although it is to be understood that it is theory only. We think that barium is attracted to a very electro-negative metal and has a tendency to be held perhaps chemically just as in a vacuum tube hydrogen is very strongly attracted by platinum; that is, a very low work function material is attracted to a high work 10 function material. This first coating of barium is poisoned and does not emit. However, when a fresh coat arrives to cover the first coating of barium it is not poisoned because the effect of the tungsten has been neutralized by combining with 15 the first coat of barium. If, instead of pure metal, a compound of the metal and another element of relatively high work function is used, the barium has less tendency to be attracted and retained chemically and if it is retained, it would probably 20 displace one of the materials which would remain on the surface and poison the barium or any other barium which may arrive.

We claim:

1. A grid structure coated with poisoning material comprising amorphous tungsten oxide. 25
2. A gaseous discharge tube comprising a cathode, anode and grid and means comprising amorphous tungsten oxide adhering to the grid for poisoning evaporated emitter material from 30 the cathode.
3. A grid structure coated with the amorphous oxide of a high work function metal. 35
4. A discharge tube comprising a gaseous conducting medium, a cathode, anode and a grid comprising means for concentrating the discharge from the cathode to the anode, and a coating of poisoning material on the grid. 40
5. The method of preventing grid emission in a gaseous discharge tube which consists in concentrating the discharge from cathode to anode and feeding poisoning material to the grid. 45
6. A controlled grid rectifier tube comprising a gaseous conductive medium, an electron emissive cathode, an anode, a grid having a perforate portion adapted to concentrate the current therethrough and having a heat radiating portion surrounding said perforate portion, and a compound of a high work function metal on said perforate portion. 50
7. A grid coating for a gas-filled, grid controlled rectifier comprising a compound of a highly electro-negative metal and another element of relatively high work function, the said compound being poisonous to the emission of highly electro-positive substances. 55
8. A discharge tube comprising a gaseous conducting medium, an oxide coated cathode, an anode, a grid having a discharge opening, said grid opening being small in size relative to the discharge current to pass through the grid whereby the discharge is concentrated through said opening, and means for disintegrating and feeding poisoning material from the anode to the grid 60 during operation of the tube. 65

EARL K. SMITH.  
DONALD V. EDWARDS.